

No. 717,864.

PATENTED JAN. 6, 1903.

J. T. JONES.

METHOD OF TREATING ORES,

APPLICATION FILED DEC. 2, 1901.

NO MODEL.



Witnesses:

Geo. S. Payard  
Geo. C. Division.

Inventor:  
John T. Jones,  
By Dyerforth, Dyerforth & Lee,  
Atty's.

# UNITED STATES PATENT OFFICE.

JOHN T. JONES, OF IRON MOUNTAIN, MICHIGAN.

## METHOD OF TREATING ORES.

SPECIFICATION forming part of Letters Patent No. 717,864, dated January 6, 1903.

Application filed December 2, 1901. Serial No. 84,436. (No specimens.)

*To all whom it may concern:*

Be it known that I, JOHN T. JONES, a citizen of the United States, residing at Iron Mountain, in the county of Dickinson and State of Michigan, have invented a new and useful 5 Method of Treating Ores, of which the following is a specification.

My invention relates to an improved method of bringing about the thorough subjection of 10 a mass of ore to the action of a chemical fluid of less specific gravity than the ore to treat the latter.

While my improved method may be advantageously employed in the treatment of 15 various ores to dissolve out the values or bring about chemical reactions, it is more especially designed for hastening and rendering thorough the subjection of the copper in copper-bearing ores to the leaching action of sulfuric acid.

In the accompanying drawing I show apparatus of simple construction which may be employed in the practice of my method.

The view represents in cross-section a vessel or barrel A of special construction supported to rotate on rollers B B. To render the practice of the method as economical as possible, the barrel should have comparatively great capacity. It may be constructed 25 with an internal diameter of, say, ten feet and be, say, sixteen feet in length, adapting it to the treatment of, say, ten tons of the ore in a single charge. The construction shown is formed of heavy oak staves a, reinforced with heavy iron hoops b and lined around its inner circumference throughout 30 with blocks C, held firmly in place, as by means of bolts c. The blocks C project inward from the circumferential wall of the 35 barrel and are formed with concave sides, presenting dippers facing in one direction around the interior of the barrel. In one side of the 40 barrel is a filling and discharging opening d, which may be tightly closed with a suitable 45 removable plug. The blocks C should be of a material or faced with a material—such as fire-clay, porcelain, or the like—which will be durable and withstand any deleterious 50 action of the acids used in the treatment of the ore.

In treating copper-bearing ores with sulfuric-acid gas in accordance with my method

the barrel is half filled—say to the line x—with the pulverized ore mixed with water to form a pulp. A hose communicating with a 55 sulfurous-acid-gas supplier is then inserted through the opening d to fill out the space above the pulp with the gas. The gas being of greater specific gravity than the atmosphere displaces the same and forces it out 60 through the opening d until the filling is completed. A plug is then inserted to close the opening d, and the barrel is rotated slowly in the direction of the arrow. In the movement of the dippers they rise at one side from the 65 pulp filled with a portion thereof, and in their movement to the highest point they discharge the pulp gradually and cause it to fall through the body of sulfurous-acid gas. As the dippers descend into the pulp on the opposite 70 side they carry down sulfurous-acid gas and discharge it gradually as they descend toward the lowest point. The gas being lighter than the pulp will rise through the pulp as fast as it is discharged from the descending dippers. 75 The simultaneous spraying of the pulp through the body of the gas and rise of gas through the mass of pulp quickly brings about a thorough subjection of the entire mass of pulp throughout to the action of the 80 sulfurous acid.

In the treatment of copper ores with sulfuric acid it is desirable, if not necessary, to prevent the formation of sulfuric acid or copper sulfate, and this is rendered possible 85 by maintaining the charge at a temperature below about 42° centigrade. The pulp and sulfurous acid when placed in the barrel or vessel should have a temperature of, say, 16° centigrade or under, whereby the chemical 90 reactions resultant upon the use of the amount of gas employed in a single charge would not raise the temperature above 42° centigrade. In case the pulp has not been treated by a single charge of the sulfurous gas sufficiently 95 to leach out the copper a hose or pipe from a chilled-air supplier may be inserted through the opening d to discharge the refrigerating fluid into the barrel until the pulp has been sufficiently cooled down, when it may again 100 be treated with a fresh charge of sulfurous acid, as before. If desired, refrigerating pipes of suitable material may pass through the barrel or be embedded in the lining C

thereof to keep the temperature of the contents of the barrel at all times sufficiently below 42° centigrade. The step of cooling or maintaining cool the contents of the barrel 5 is a desirable feature of my improved method when applied to the treatment of copper ore with sulfurous acid, as described. However, the tendency toward the production of sulfuric acid at a temperature above 42° centi- 10 grade makes it possible, when desired, to make a sulfate by dispensing with the refrigerating step.

What I claim as new, and desire to secure by Letters Patent, is—

15 1. The process of mixing with ore, to be treated, a leaching fluid, which consists in confining the mass of ore in a vessel with a body of leaching fluid of lesser specific gravity superimposed upon it, carrying portions 20 of the ore upward in said vessel and releasing it above the body of leaching fluid to precipitate it through said body, and simultaneously conveying portions of the leaching fluid below the surface of the mass of ore and releasing it and permitting it to rise through 25 the same.

2. The process of mixing with ore, to be treated, a leaching fluid, which consists in

confining the ore in the condition of pulp in a vessel with a body of leaching fluid of lesser 30 specific gravity superimposed upon it, carrying portions of the pulp upward in said vessel and releasing it above the body of leaching fluid to precipitate it through said body, and simultaneously conveying portions of the 35 leaching fluid below the surface of the mass of pulp and releasing it and permitting it to rise through the same.

3. The process of mixing sulfurous-acid gas with copper ore in the condition of pulp, 40 which consists in confining the mass of pulp in a vessel with a body of sulfurous-acid gas superimposed upon it, carrying portions of the pulp upward in said vessel and releasing it above the body of gas to precipitate it 45 through said body, simultaneously conveying portions of the gas below the surface of the mass of pulp and releasing it and permitting it to rise through the same, and subjecting the pulp in the vessel to the action of a 50 cooling fluid, substantially as set forth.

JOHN T. JONES.

In presence of—

ALBERT D. BACCI,  
WM. B. DAVIES.